

Aug. 10, 1926.

1,595,838

H. W. TURNER

PREFORMED ELECTRICAL COIL

Filed May 15, 1923

Fig. 1.



Fig. 2.



Inventor:  
Harry W. Turner,  
by *Alexander S. Gant*  
His attorney.

## UNITED STATES PATENT OFFICE.

HARRY W. TURNER, OF SCHENECTADY, NEW YORK, ASSIGNOR TO GENERAL ELECTRIC COMPANY, A CORPORATION OF NEW YORK.

## PREFORMED ELECTRICAL COIL.

Application filed May 15, 1923. Serial No. 639,230.

My invention relates to preformed electrical coils and has for its object the provision of a coil which is solidified without the use of auxiliary bonding agents.

In the manufacture of preformed coils of various types for electrical apparatus, it has heretofore been customary to solidify the coil after it has been wound by inserting strips of shellacked paper or fabric between the turns of the coil and then concurrently applying heat and pressure to the coil whereby the shellac was softened and when allowed to cool held the turns of the coil together in a solid mass which had been compacted by the pressure to a predetermined size. Since shellac has a great affinity for moisture, this method is obviously detrimental to the insulating properties of the coil. Thread and tape have also been used for bonding coils.

In carrying out my invention, I form the coil from a conductor covered with a fibrous insulating material which has been impregnated with a suitable non-hygroscopic adhesive insulating material, such as an asphaltum compound, and then apply suitable heat and pressure to the coil whereby the asphaltum compound softens and cements the conductors of the coil together into a solid compact mass.

For a more complete understanding of my invention reference should be had to the accompanying drawing in which Fig. 1 shows apparatus for forming electrical coils in accordance with my invention; while Fig. 2 is a section view of a coil embodying my invention.

Referring to the drawing, in one form of my invention the conductor 10 provided with a fabric insulating covering impregnated with an asphaltum compound is wound into an electrical coil 11. After being formed, the coil 11 is placed in a suitable clamping device 12 whereby the portions of the coil which are to be inserted in slots or other limited spaces in the apparatus with which the coil is to be used are compressed. At the same time the coil is heated in a suitable manner, for example, by passing an electric current therethrough by means of conductors 13 and 14 leading from a suitable source of electrical supply. The heat applied to the coil softens the asphaltum compound with which the fabric insulating material on the conductors is impregnated,

and the pressure applied compacts the coil to the required dimensions. Upon being allowed to cool the asphaltum compound acts as a cement firmly holding the conductors of the coil together so that the whole is formed into a solid compact mass, as shown in Fig. 2. I have found that the coils should be heated to approximately 140 degrees C. in order to soften the asphaltum compound sufficiently to permit it to cement the conductors together. The asphaltum compound is non-hygroscopic so that the coil is effectively sealed against the entrance of moisture.

In the treatment of the conductor 10, the asphaltum compound may and preferably is applied to the cotton or other fibrous covering of the conductor at a relatively high temperature, such as about 500 degrees F. The cotton covered conductor may be passed through a bath of the asphaltum compound maintained at the temperature referred to. At this temperature the residual moisture and air are first boiled out of the cotton and then, the viscosity of the normally solid asphaltum compound being relatively low at such high temperatures, the interstices between the fibres of the cotton and even the structure of the fibres are penetrated and filled with the dense asphaltum substance that effectively prevents the reentrance of moisture and air. For the purpose of rendering the surface more repellent to moisture and acids and the covering more pliable, a coagulable vegetable oil, such as China wood oil, may then be applied while the conductor is still hot. Such an insulated conductor is described and claimed in my copending application, Serial No. 449,943, filed March 5, 1921.

The use of shellac and other objectionable bonding agents for solidifying the coil is thus eliminated, whereby the coil has better insulating properties and may be compressed into the smallest possible space. I have found, in fact, that the conductors of the coil may be bonded together in this manner and compressed to approximately the same dimensions as a similar group of conductors provided with untreated cotton coverings. If desired, the coil may be solidified before removing it from the winding form by simply applying heat and pressure to it. By means of my invention, the process of producing coils is thus greatly simplified.

and consequently the cost of production is reduced. In short, the coil, after being wound, is solidified simply by applying heat and pressure, no bonding agent, or thread or tape for tying the conductors in place being necessary.

While I have described my invention as embodied in concrete form and as operating in a specific manner in accordance with the 10 provisions of the patent statutes, it should be understood that I do not limit my invention thereto, since various modifications thereof will suggest themselves to those skilled in the art without departing from 15 the spirit of my invention, the scope of which is set forth in the annexed claims.

What I claim as new and desire to secure by Letters Patent of the United States, is:

1. The method of making an electrical 20 coil which consists in providing a conductor having a fibrous covering, impregnating said fibrous covering by passing the conductor through a bath of molten asphaltic material heated to a temperature high enough to thinly liquefy it, winding the conductor into a coil, heating the coil thus formed to a

temperature high enough to soften the asphaltic material while applying pressure to compact the turns of said coil, and then applying said pressure while the asphaltic material cools and hardens whereby said turns are bound together into a solid mass by said asphaltic material.

2. The method of making an electrical coil which consists in providing a conductor having a coating of fibrous insulating material, passing said conductor through a bath of molten asphaltum heated to a temperature of approximately 500° F. whereby said fibrous coating is thoroughly impregnated with said asphaltum, winding said conductor into a coil, heating the coil thus formed to a temperature of approximately 284° F. to soften said asphaltum, compacting the turns of the coil while the asphaltum is softened, and then maintaining the turns compacted while said asphaltum cools and hardens whereby said turns are bound together by said asphaltum into a solid mass.

In witness whereof, I have hereunto set my hand this 11th day of May, 1923.

HARRY W. TURNER.